

## UNITED STATES PATENT OFFICE

2,038,208

## PROCESS OF HEAT TREATING METALS

William E. Day, Jr., Plainfield, N. J., assignor to  
 International Motor Company, New York, N. Y.,  
 a corporation of Delaware

No Drawing. Application March 23, 1933,  
 Serial No. 662,295

4 Claims. (Cl. 148—21.5)

The present invention relates to methods for heat treatment of axles, shafts, etc., and embodies, more specifically, an improved method of heat treatment by means of which the strength 5 of the objects so treated under torsion is greatly increased.

It is known that the stresses in a shaft or member undergoing pure torsion may be resolved into two components of shear, one of tension and one 10 of compression. These stresses are greatest at the surface of the object and zero at its axis. Since these stresses are in equilibrium up to the elastic limit of the material, failure will occur due to the relative shear and tensile properties in the 15 material along the lines in which these stresses lie. In shafts which are produced either by rolling or forging a weakness exists in the direction of the axis due to the preferential orientation of slip planes (the planes represented by the less 20 densely packed atoms in the primary crystal). The flow lines, in general, after severe working, follow the direction of the slip planes. These lines, however, cannot be destroyed by any sort of treatment, whereas the slip planes may be 25 made by the treatment described herein, to change their direction. It has been found that this structure of the metal cannot be completely broken down even after long periods of annealing. This weakness in shafts may be intensified 30 by certain heat treatments and eliminated by others. In general, treatments producing extreme hardness aggravate this condition.

By the method described herein, the preferential orientation of slip planes is definitely eliminated and the section of the shaft adjacent the surface is treated to produce extreme fitness therein with no brittleness. The treatment further produces a shaft having a core of relatively high strength but nevertheless possessed of ductility and free from brittleness.

The strength of steel in torsion members, particularly in shafts heat treated by methods now in practice, does not exceed 160,000 pounds per square inch and in most cases is considerably less 45 than this value. This refers to the maximum shear stress which is taken as the maximum torsional moment over the polar section modulus. All attempts to increase this value by heat treating to greater hardness have failed because the 50 material develops directional weakness when so treated by conventional methods, the shaft rupturing by splintering frequently at extremely low values.

In accordance with the heat treatment of the 55 present invention, the directional weakness is

overcome and the permissible shear stress is raised to values exceeding 200,000 pounds per square inch. Furthermore, the method in accordance with the present invention produces a strength gradient which is a maximum at the 5 outer fibre of the shaft, thus producing a condition which is in accord with the theory noted above as to shafts in torsion. Shafts which have been treated in accordance with the present invention frequently require three times more work 10 to rupture them in torsion than is the case with shafts which are treated in accordance with common practice.

The method comprised by the present invention is particularly applicable in the treatment of 15 shafts made from steels of analyses such that when subjected to a hardening heat treatment and tempered they will possess a martensitic or martensito-troostitic structure, and, more particularly, those alloy steels known as pearlitic-martensitic steels, of which the chrome-nickel steel referred to hereinafter is a representative example.

According to the method of the present invention, a steel shaft of a suitable analysis is heated 25 until the temperature throughout is slightly in excess of its upper critical point (hardening point). The shaft is then quenched. The shaft, which has now been hardened throughout, is then tempered by reheating to a tempering temperature and quenching from such temperature, the tempering temperature being such as to retain the steel in a martensitic state. After this preliminary treatment, the shaft is heated rapidly until the temperature in the surface portions has 30 been brought above the upper critical point while controlling the rate of heat input and time of heating so that the core is heated to a temperature slightly below the upper critical point, thereby insuring that the carbides in the surface layer 35 are substantially completely absorbed by the gamma iron and the carbides in the adjoining layers are more or less completely so absorbed. The shaft is then quenched. The time of heating and the temperature of the heating medium 40 must be consistent with the section and analysis of the material undergoing treatment. After the foregoing operation, the shaft is drawn by reheating to a temperature between 300° F. and 45 400° F. to remove strains.

A specific illustration of this method is as follows:

A shaft 36" long and 1.6875" in diameter throughout its body, having its ends splined for a distance of 3.5" and of a diameter at this 55

point of slightly over 2", consisting of material comprising 3.5% nickel, 1.30% chromium, .35% carbon, .02% phosphorus, .02% sulphur, and the balance of iron, is first properly annealed and then heated to 1425° F. The shaft is quenched in oil and reheated to 800° F. and quenched in water. The foregoing steps are in accordance with common practice. The shaft is then immersed in a lead bath for 90 seconds, the temperature of the bath being 1800° F. It is then quenched in oil and drawn at 425° F. The time of heating in the 1800° F. bath for shafts of larger diameter must necessarily be increased. For example, a shaft of 1.9" in diameter must be heated for 100 seconds in accordance with the factors outlined hereinafter.

To determine the proper length of time during which a shaft is subjected to the lead bath, in the case of a circular shaft, the following differential equation, given by Carslaw in "The Conduction of Heat" at page 222, is solved, the temperature at any point from the axis of the shaft being dependent upon its radius and the time factor.

$$25 \quad \frac{\partial v}{\partial t} = K \left( \frac{\partial^2 v}{\partial r^2} + \frac{1}{r} \frac{\partial v}{\partial r} \right)$$

The solution of this equation is given by Carslaw as:

$$30 \quad v = V_0 \left[ 1 + \frac{2}{a} \sum_{n=1}^{\infty} \frac{J_0(\alpha_n r)}{J_0(\alpha_n a)} \frac{e^{-\alpha_n^2 k t}}{\alpha_n} \right]$$

In the foregoing equation:

$V$ =temp. at a

35  $V_0$ =temp. at surface  $r=a$

$a$ =radius

$k$ =constant of diffusivity

$t$ =time

The summation is taken over the positive 40 roots of

$$J_0(\alpha a) = 0$$

In ordinary problems of heat diffusion

$$45 \quad k = \frac{K}{c\rho}$$

where  $K$  is the conductivity and  $c$  and  $\rho$  the specific heat and density, respectively. In medium carbon steel the numerical value of 50  $k = .121$  C. G. S. units. The use of this value is permissible up to a point where the critical range of the steel is reached. At this point a sharp change in the specific heat takes place with a corresponding change of heat absorption due to 55 the change of the metal from the alpha to the gamma state. The mean value of  $k$  as determined under this condition through experimental means is found to be .0135. The use of this value in the above equation together with the other 60 proper substitutions, and then solving for  $t$  gives the required time.

Solution for a shaft 1.6875" diam.  $a = 2.14$  cm.

Desired temp. center=482° C.

Desired temp. outside=815° C.

$$65 \quad k = .0135$$

Substituting in (1)

$$482 = 815 \left[ 1 + \frac{2}{2.14} \left( \frac{1}{-51} \right) \frac{e^{-0.0135 \times 1.31 \times t}}{1.143} \right]$$

$$70 \quad t = \frac{\log \frac{1310}{333}}{.434 \times .0135 \times 1.31} = 90.5 \text{ sec.}$$

The foregoing solution is accurate where the 75 heating time is such that the critical point of the

steel is not exceeded for any long period of time. The permissible shear stress of shafts treated in this fashion is 40% greater and the ultimate angle of torsion twice as great as in shafts treated in accordance with existing methods. If 5 the permissible fibre stress is exceeded the failure will consist of a clean shear at right angles to the axis of the shaft, and will not be of the dangerous splintering or helicoidal type, common in hard shafts which are conventionally heat treated. 10 The following tabulation illustrates the characteristics of shafts treated in accordance with the present invention and affords a comparison between the shafts produced by the old method and those produced in accordance with the present invention. 15

| Torsional moment              | Old shaft             | New shaft |
|-------------------------------|-----------------------|-----------|
| 1. At elastic                 | 115,000#"             | 120,000#" |
| 2. At ultimate                | 152,000-<br>156,000#" | 210,000#" |
| 3. Angle at elastic limit     | 21°                   | 41°       |
| 4. Angle at ultimate strength | 180,200°              | 400-500°  |

25

It will thus be seen that shafts treated in accordance with the present invention have at least 25% more torsional capacity and are able to resist at least twice as much shock as shafts treated in accordance with the present methods.

Although the foregoing has referred to the treatment of shafts, the method of the present invention is well suited to the hardening of springs and other elements subjected to bending by reason of the high strength produced in the surface layers by the improved method and the lack 35 of brittleness of the said layers.

While the invention has been described in connection with the heat treatment of a shaft having the characteristics noted herein, it is 40 not to be limited, either as to the nature of the objects treated, nor as to the specific method of treatment, save as defined in the appended claims.

I claim as my invention:—

1. The process of heat treating structural steel 45 parts made from steels of the pearlite-martensitic type to increase their resistance to impact and torsional stresses which comprises subjecting such a part to a hardening heat treatment wherein the said shaft throughout its section is heated above the upper critical range of the steel and then quenched, then subjecting said part to a tempering heat treatment followed by quenching to place the steel in a predominantly 50 martensitic state throughout, heating the thus treated part to bring the temperature in its surface portions above the upper critical range while controlling the rate of heat input and time 55 of heating so as to create a temperature gradient inwardly from the outside of the part such that the core and the innermost layers are heated slightly below the upper critical range, and then quenching.

2. The process of heat treating steel shafts and the like made from steels of the pearlite-martensitic type to increase their resistance to torsional stresses which comprises subjecting such a shaft to a hardening heat treatment wherein the said shaft throughout its section is heated 60 above the upper critical range of the steel and then quenched, then subjecting said shaft to a tempering heat treatment followed by quenching 65 to place the steel in a predominantly martensitic state throughout, heating the thus treated 70

75

- shaft to bring the temperature thereof in its surface portions above the upper critical range while controlling the rate of heat input and time of heating so as to create a temperature gradient along the radii of the shaft such that the core and the innermost layers are heated slightly below the upper critical range, and then quenching, thereby hardening the outer layers while promoting a tempering of the core and inner layers.
3. The process of heat treating steel shafts and the like made from a pearlite-martensitic chrome-nickel steel to increase their resistance to torsional stresses which comprises subjecting such a shaft to a hardening heat treatment wherein the said shaft throughout its section is heated above the upper critical range of the steel and then quenched, then subjecting said shaft to a tempering heat treatment followed by quenching,
- 20 heating the thus treated shaft in a lead bath until its surface portions have been brought above the upper critical range, and then, while the temperature of the core is still below the upper critical range, quenching the shaft in oil, and finally reheating to a moderate temperature below the lower critical range to remove strains.
4. As an article of manufacture, a heat treated structural steel part made from a pearlite-martensitic steel and having a hardened and tempered core in supporting relation to an overlying hardened outer portion, said part being made by subjecting the same to a hardening heat treatment wherein the said shaft throughout its section is heated throughout the upper critical range of the steel and then quenched, then subjecting said part to a tempering heat treatment followed by quenching to place the steel in a pearlite-martensitic state throughout, heating the treated part to bring the temperature in its surface portions above the upper critical range while controlling the rate of heat input and time of heating so as to create a temperature gradient inwardly from the outward side of the part so that the core and the innermost layers are heated to the upper critical range of the steel, and then quenching.

WM. E. DAY, JR.